

# UNITED STATES PATENT OFFICE.

HENRY M. HOWE, OF BEDFORD STATION, NEW YORK, ASSIGNOR TO TAYLOR-WHARTON IRON & STEEL COMPANY, OF HIGH BRIDGE, NEW JERSEY, A CORPORATION OF NEW JERSEY.

## MANUFACTURE OF STEEL ARTICLES.

1,123,193.

Specification of Letters Patent.

Patented Dec. 29, 1914.

No Drawing. Application filed July 17, 1909, Serial No. 508,113. Renewed July 9, 1914. Serial No. 850,054.

To all whom it may concern:

Be it known that I, HENRY M. HOWE, a citizen of the United States of America, residing at Bedford Station, in the county of 5 Westchester and State of New York, have invented certain new and useful Improvements in the Manufacture of Steel Articles, of which the following is a full, true, and concise specification.

10 The purpose of the present invention is the production of an integral steel article having a hardened exterior part or surface especially adapted to resist abrasion or wear, and a tough or ductile interior especially 15 adapted to resist strain or shock, so that the article as a whole is adapted to resist simultaneously both wear and shock and in a superior degree.

20 The invention is not concerned with the shape or nature of the steel article and may be applied to any steel article wherein these properties are of value; as, for example, to 25 steel gear-wheels or pinions which are required to sustain strain and shock generally while their teeth and bosses are specially required to resist wear, or a ring or cylinder needing a hard inner surface. With such an 30 article, or any article, my invention contemplates the formation of the surface of the article or the part or parts which are to be subjected to the wearing action, of steel alloy in the condition or state known as martensite, and the remainder of the article, that is to say, its body or the interior parts 35 not intended to resist wear, of steel alloy in the condition or state of austenite. By the term "steel alloy" I refer to all alloys of iron, other than the common white cast iron and gray cast iron. There is no general 40 agreement as to the distinction between cast iron and steel, and there may be some persons who would call certain of the alloys to which I refer "cast iron," while others would call them "steel." The essential thing in all 45 of them is that they are capable of being made at will in part austenitic and in part martensitic.

As is known to those skilled in this art, there are three well marked states or conditions of steel alloys of the kind referred to; (1) austenite, the normal non-magnetic condition existing spontaneously at and above a bright red heat; (2) pearlite, the

common magnetic state, in which all our 55 common slowly cooled iron and steel objects exist; and (3) martensite, an intermediate state. When steel is heated to above a certain critical temperature called  $Ac_3$  and which varies from about  $500^{\circ}$  C. to about  $900^{\circ}$  C. with the composition of the steel, it 60 passes spontaneously into the austenite state.

In cooling the austenite in general passes spontaneously either first into martensite and then into pearlite, which is the common 65 constituent of annealed carbon steel, or it may pass directly into the pearlite state, skipping over the martensite state. The temperature at which such steel becomes austenite when the temperature is rising is called  $Ac_3$ , and the temperature at which it 70 passes out of the austenite state when the steel is cooling is called  $Ar_3$ . This  $Ar_3$  temperature is habitually somewhat lower than  $Ac_3$ , and, in case a very large percentage of nickel is present it may be very far 75 below  $Ac_3$ . When the steel alloy contains a relatively large percentage of the elements manganese and nickel which I term obstructive elements because they obstruct the escape from the austenite and martensite 80 conditions, these conditions have a relatively firm stability and remain austenite or martensite as the case may be notwithstanding that their cooling may occur very slowly and every opportunity given for the change to 85 take place, but where the proportions of these elements are less, the alloy tends to undergo transition through the successive stages above mentioned. By quickly cooling steel alloy of the kind just referred to while 90 in the condition of austenite, as by quenching it from far above  $Ac_3$  in cold water, the austenitic formation or condition may be preserved in a state of stability which, though not complete, is sufficient for many 95 practical purposes. The rapidity with which the steel cools through the range of temperature in which it is liable to shift from the austenite state into first that of martensite and from this into that of pearlite, (the temperature below  $Ar_3$ ) increases 100 with the temperature at which the steel is at the moment of quenching. The higher the quenching temperature the faster does the steel cool through this range. Hence in order 105 that the cooling through this range

should be extremely rapid and that the quenching should have the greatest effect in fixing the austenite state, the steel when quenched should be at a temperature far above  $Ac_3$ . For instance, quenching small steel objects containing 2 per cent. of carbon and 2 per cent. of manganese in ice water from  $1050^{\circ}$  C. preserves them in the austenite state, whereas quenching from a temperature which though still above  $Ac_3$  is yet much below  $1050^{\circ}$  C. would leave them in the martensite state. In the same way cooling them less rapidly, but still rapidly, from  $1050^{\circ}$  C. would leave them in the martensite state, and cooling them slowly would leave them in the pearlite state. Such lower temperatures may be called martensitogenous and pearlitogenous respectively. The rate of cooling necessary to fix these conditions is known to the art, but quenching in a cold liquid is the most practical method. The presence of carbon adds to the obstructive effect of the elements, manganese and nickel.

In many cases the austenite thus produced and fixed is not pure but is mixed with martensite, and in other cases the martensite is diluted with austenite. Therefore when I speak of steel in the austenitic state I do not refer solely to absolutely pure austenite, but I also include steel in which the proportion of austenite to martensite is such that the properties of the steel as a whole are due in chief part to its austenite, perhaps unavoidably or even in some cases advantageously modified by the accompanying martensite. So with my references to the martensitic state, *mutatis mutandis*. These conditions of steel alloys are readily distinguished and are well known to those skilled in the science of metallurgy; generally they are regarded as different chemical or mechanical combinations or solutions of the same elements of which the alloy has been prepared in the first instance.

Austenite is ductile or more accurately is shock-resisting. As usually known, in the steels very rich in manganese and nickel, it is also very much harder than common steel in its annealed state, though less hard than hardened steel. But this hardness is probably due to the presence of the nickel and manganese respectively, because when steel poor in manganese and nickel is brought to the austenitic state it is relatively soft. The hardness of such austenitic steel as determined by the Shore scleroscope, is about that of annealed wrought iron. In the majority of cases included in this invention the austenite is hard. But its chief value lies in its power of resisting shock abrasion. It resists shock better than martensite. It resists abrasion better than pearlite, but not as well as martensite. Austenite is non-magnetic (in the sense of being very feebly magnetic), and appears under

the microscope in irregular polygons. The ordinary manganese steel of commerce containing about 12% manganese and  $1\frac{1}{2}$ % carbon is an example of steel alloy consisting almost entirely of austenite, and another example is found in ordinary nickel steel containing about 25% nickel. Martensite on the other hand, is much harder than austenite, more brittle, and appears under the microscope in the form of interlacing streaks or needles forming angular or triangular markings. Generally compared, the difference between martensite and austenite is of the same kind as that between the case-hardened and the non-case-hardened parts of a soft steel object, though the former difference is less marked than the latter. A combination of the austenitic and the martensitic states in one and the same object is more easily obtainable in steels containing lesser percentages of manganese or of nickel than just above stated.

In carrying out my invention I form the article in the first instance by casting, forging or otherwise, of steel or iron alloy of the kind referred to; that is to say, having a composition which makes it capable of existing in the states of austenite and martensite. I then treat the article according to one of several methods so as to produce the martensitic condition in the part which is to be made wear-resistive, and the austenitic condition in the rest of the article. The means by which I do this are either (1) to manipulate the temperature of the different parts so as to produce austenite in the one part and martensite in the other; or (2) to shift the metal in part of the object into the martensite state by mechanical deformation; or (3) to vary the composition relatively in the two parts so as to make one part so rich in the obstructive elements, manganese, nickel and carbon that it may remain as austenite, and the wear-resistive part less rich in these obstructive elements so that it may slip into the martensite state under proper treatment. Or I may combine these different methods, using each to reinforce the effect of the other.

The methods numbered (1) and (2) are evidently chiefly applicable to metal with a marked but yet controllable degree of instability. The third is chiefly applicable to metal which has initially such an intermediate degree of instability, *i. e.* an intermediate percentage of the obstructive elements that it is practicable, by locally changing the composition within practicable bounds, to produce useful differences in the degree of instability. In this way part of the metal may be so unstable that it slips into the martensite state, while the rest is so stable that it can be held in the austenite state. But I often reinforce the effects of local

differences in composition by intentional differences in thermal treatment and in mechanical deformation.

In the case of the gear-wheel or pinion, 5 the surface of the teeth is converted into martensite and the remainder into austenite. The method by which I prefer to produce the transformation in case of small pinions, and which I now proceed to describe, is to 10 quench the whole pinion from a temperature high enough to cause the whole of it to remain austenitic, and then to reheat the surface or wearing parts to a temperature at which they become martensitic, and then 15 again to quench the whole, lest the change go too far and either too much of the austenite changes into martensite, or too much of the martensite changes into pearlite. In this way I fix the conditions of austenite 20 and martensite in the respective parts in which they are severally needed. For example, the article made of say manganese steel containing 2% manganese and 2% carbon, is first brought throughout its mass to 25 a temperature well above the point  $Ac_3$  or say to  $1050^{\circ} C.$ , it being understood that the actual temperature of  $Ac_3$  will vary somewhat with the nature and ingredients of the steel alloy, and that the temperature actually 30 reached may vary in different parts of the piece, provided that is well above  $Ac_3$ . The point at which a particular steel becomes austenite, however, is well known and easily determinable by those skilled in this art. 35 The article is then plunged in ice water, in the way practiced in the treatment of the ordinary manganese steel of commerce, except that for this specific composition the cooling should progress the more rapidly, 40 with the result that the entire article becomes austenite. I thereupon expose the article, or those portions of it which are to be made of martensite, to a degree of heat and for a short time, but sufficient to raise or 45 bring the temperature of the surface for a depth of about one-sixteenth of an inch more or less up to or above a temperature at which the particular steel alloy is known to shift over into the martensitic state. This 50 temperature is always lower for a given alloy than that which produces austenite, and like that temperature it may be determined beforehand with a sample of the alloy or after some experience may be gaged 55 roughly with the known alloy by the oxid color or the glow color as the case may be. An example of the time and temperature for a very small steel pinion having the above composition would be to heat its surface 60 quickly to  $400^{\circ}$ , keeping the interior as nearly cool as practicable. By the glow color I refer to the colors such as dark blood red, cherry red, etc., caused by the glowing of the object, as distinguished from the oxid 65 colors.

During the heating of the article, it will be well to protect it against oxidation. With the surface thus transformed to the martensitic condition, the article is again quickly cooled, as by plunging it into cold water, and thereby the martensitic condition becomes fixed in the surface of the article or in such parts thereof as have been subjected to the surface heat and are desired to resist wear. The remainder is austenite, 70 integrally joined to the martensite. While of itself a brittle and glassy-hard material, the martensite thus produced is disposed on the surface of the article for a slight depth only, say one-sixteenth of an inch, and is so supported by the body of the austenite underneath it and into which it merges, that its natural tendencies to crack or splinter under shock or blows are quite avoided and the article as a whole is exceedingly durable 75 and capable of long wear. A useful composition for treatment in this manner may consist of manganese steel containing from 6 per cent. of manganese and .85 per cent. carbon to 9% manganese and .75% carbon, intermediate percentages of manganese being used with proportional amounts of carbon. 80

Instead of first producing a uniform condition of austenite throughout the entire body of the article, it may be heated at one 85 and the same time up to an austenitogenous temperature and then the surface may be allowed to cool to a martensitogenous one, and then by a single quenching it may be preserved in these respective states. This I 90 call a differential quenching. If a certain part only of the article is required to be hard and wear-resistive, *i. e.* of martensite, all the rest of it may be heat-insulated so as to retard the cooling except as to that 95 part which is left exposed and thus air cools more rapidly than the rest of the article (but, of course, cooling at a rate incomparably less than that needed to retain austenite). When the faster cooling part has 100 reached the martensitogenous temperature, but while the slower cooling part is still in the austenitogenous range of temperature, these conditions are fixed in them by a single 105 quenching. 110

Conversely, during the heating process the part or parts to be made of martensite may be heat-insulated or may be made thicker than the rest of the article exposed, whereby the two parts reach respectively the 115 martensitogenous and austenitogenous temperatures at about the same time or can be readily brought to such temperatures so that a single rapid cooling will fix these states and complete the process. If the heating 120 under such conditions should produce in the more exposed part a temperature unduly above that of the rest, its exposed condition will permit it to cool more rapidly than the insulated parts, so that proper tempera- 125 130

tures will be ultimately and simultaneously obtained in both before quenching.

A further method of producing a similar shock and wear-resistive article by a single sudden cooling and above referred to, consists in forming the article uniformly of austenitic steel, and then, after it is established as such, deforming the surface of the article which is to be made wear-resistive, as by rolling, swaging or drawing it. This may be done in the cold. In such cases the quantity of the obstructive elements should be only moderately above the minimum required for maintaining the austenite state by quenching, (a point which varies but is determinable) so that that state will be sufficiently unstable to enable it to shift over into the martensitic state simply by the mechanical deformation of rolling or otherwise working the surface of it, and without further heat treatment.

The effect of mechanical deformation is, as I believe, to relieve the pressure existing in the surface of the article. Pressure coöperates with the obstructive elements, carbon, manganese, and nickel, to retain the metal in the austenite state; and tension or the release of pressure opposes them and favors the passage into the martensite state, for the reason that martensite is more bulky than austenite. The deformation which occurs for example in cold rolling produces local tensions at time, alternating with local pressure. When the pressure is released or turned into tension the obstructive elements, no longer reinforced by the pressure, may not suffice to hold a steel of moderate instability in the austenite state, and it will in that case shift into the martensite state. But the restoration of the pressure locally will not return the metal to the austenite state. Hence the alternations of pressure and tension which occur during cold deformation have the effect of changing austenite into martensite.

A still further method consists of forming the article of a steel alloy capable of stable or fairly stable austenitic condition by reason of the proportions of its obstructive elements, and then by chemical action lessening the proportion of these elements on the surface or on the parts to be subjected to wear, so as to bring about conditions which give rise to martensite and thereafter quickly cooling the article by a single quenching. For instance, a given percentage manganese steel with a moderate quantity of carbon shifts more readily from the austenitic into the martensitic state than steel with more carbon. Hence, if a steel article containing enough carbon and manganese jointly to cause the retention of the austenitic state during a given treatment be superficially decarburized to a moderate extent by any usual method, for instance by heating it in

contact with iron oxid, the outside of that object may be then shifted over into the martensitic state while the inside remains in the austenitic state. When such an object is cooled quickly from say 1100° C., the outside will in cooling become martensitic, while the inside remains austenitic. If the cooling is so sudden as to retain even the outside in the austenitic state, then on slight reheating the outside will become martensite. An example of this method would be to heat manganese steel articles of 8.4% manganese and 1.3% carbon, at say 950° C. for twelve hours in contact with iron oxid and sand and then raise it to 1100° C. and quench in cold water.

I claim the following:

1. An integral wear and shock resistive steel article having its wear surface made of steel in the condition of martensite and the remainder or body portion of steel in the condition of austenite.

2. An integral wear and shock resistive article formed of an alloy of manganese, iron and carbon, and having its wear surface fixed in the condition of such alloy known as martensite and the remainder in the condition of austenite.

3. A wear and shock-resistive steel article having a portion of its wearing face for a depth of approximately  $\frac{1}{16}$  inch made of steel alloy in the condition of martensite and the remainder of the article of steel in the condition of austenite.

4. A method of making wear and shock resistive steel articles which consists in treating the surface portion of the article to produce therein the condition of martensite and the rest of the article to produce therein the condition of austenite.

5. A method of manufacturing surface-hard steel articles which consists in forming the article of a steel-alloy capable of the austenitic condition and subsequently treating the article to produce the martensitic condition on its surface and the austenitic condition throughout its interior.

6. A method of manufacturing surface-hard steel articles, which consists in forming the article of a metallic alloy capable of existing in the states of austenite and martensite and subjecting the surface and interior of the said article to sudden cooling from temperatures respectively adapted to produce the martensitic and austenitic states therein.

7. A method of manufacturing wear and shock-resistive steel articles which consists in forming the article of manganese steel containing upward of five per cent. manganese, and subjecting the surface parts desired to be wear resistive, and the remainder of the article, respectively, to sudden cooling from temperatures respectively adapted to produce the martensitic and austenitic states therein.

austenitic conditions of manganese steel therein.

8. A method of manufacturing wear and shock resistive steel articles, consisting in  
5 making the article of steel alloy capable of existing as austenite and martensite, cooling the article from an austenite producing temperature to fixate such condition therein, reheating the surface of the article, with  
10 sufficient application of heat and for a sufficient period to cause only a surface portion

of moderate depth to shift over to the state of martensite and then fixating such state by cooling the article.

In testimony whereof, I have signed my 15 name to the specification in the presence of two subscribing witnesses.

HENRY M. HOWE.

Witnesses:

HELEN M. TOWER,  
H. G. KIMBALL.